# EUROPEAN PATENT SPECIFICATION

(11) **EP 2 361 188 B1**
(45) Date of publication and mention of the grant of the patent: **08.05.2019**
(21) Application number: 09759730.6
(22) Date of filing: 24.11.2009
(51) Int. Cl.: B42D 25/369, B42D 25/387, B42D 25/364, B42D 25/41, B42D 25/382, B42D 25/45, B42D 25/378

(54) **MAGNETICALLY ORIENTED INK ON PRIMER LAYER**
MAGNETISCHE AUSGERICHTETE FARBE AUF EINER HAFTSCHICHT
ENCRE MAGNÉTIQUEMENT ORIENTÉE SUR UNE COUCHE D'APPRÊT

(30) Priority: 24.11.2008 WO PCT/IB2008/003192
(43) Date of publication of application: 31.08.2011
(73) Proprietor: SICPA HOLDING SA, 1008 Prilly (CH)
(72) Inventor: DESPLAND, Claude-Alain, CH-1008 Prilly (CH); SCHMID, Mathieu, CH-1005 Lausanne (CH); VEYA, Patrick, CH-1131 Tolochenaz (CH)
(74) Representative: Hoffmann Eitle
(86) International application number: PCT/EP2009/065731
(87) International publication number: WO 2010/058026

(56) References cited:
- EP-A1- 1 669 213
- WO-A-2007/131833
- WO-A2-03/089250
- WO-A2-2009/074284
- US-A1- 2003 232 210

## Description

### Field of the Invention

The present invention is in the field of security document printing. It concerns in particular an improvement to an ink-based security element, which is obtained on a fibrous or otherwise porous substrate through printing and magnetically orienting an ink comprising magnetic or magnetizable pigment particles, as well as the production and the use of said security element, and security documents carrying said security element.

### Background of the Invention

Security elements and decorative coatings containing oriented magnetic particles in a printed and cured ink layer, and methods for producing and for using them, are known from US 3,676,273; US 3,791,864; EP 406,667 B1; EP 556,449 B1; EP 710,508 A1; WO 02/90002 A2; WO 2005/002866 A1; WO 2006/061301 A1; WO 2006/117271 A1; WO 2007/131833 A1; as well as from the applications EP 1 880 866 A1 and WO 2008/046702 A1. Particularly useful in this context are optically variable magnetic pigments, such as disclosed in US 4,838,648; in EP 686,675 B1; in WO 02/73250 A2 and in WO 03/00801 A2, WO 2004/024836, and the methods for orienting said pigment in the printed ink, disclosed in EP 1 810 756 A2, WO 2005/002866 A1, WO 2006/069218, in the co-pending application WO 2008/046702 A1, and in the hereto related documents.

According to WO 2005/002866 A1, predetermined indicia, such as lettering, a design, or an image, are magnetically transferred onto a printed document, i.e. a sheet or a web, carrying a layer of a freshly printed, wet ink or coating composition comprising magnetic or magnetizable particles (F), through the exposition of said sheet or web to a plate of permanent-magnetic material which carries said predetermined indicia in the form of engravings in its surface, hereby orienting the magnetic or magnetizing particles (F), followed by curing (hardening) the ink or coating composition so as to immobilize the oriented magnetic or magnetizable particles (F). Patent application WO 2008/046702 A1 is about a further improvement to the magnetic orientation device disclosed in WO 2005/002866 A1.

As disclosed in WO 2007/131833 A1, particular ink formulations are required in order to obtain a visibly appealing result. In particular, in the case of inks containing magnetic platelets, such as optically variable magnetic pigment flakes, the ratio of the volume of the (dried, solvent-free) ink vehicle to the volume of the magnetic pigment should be higher than 3.0, most preferably higher than 5.0, in order to provide enough space in the ink layer for the magnetic pigment particles to freely adopt an externally imposed orientation.

However, it was observed that the quality of the magnetically oriented image depends also to a large extent on the substrate onto which the said layer of ink or coating composition comprising said magnetic or magnetizable particles (F) is applied. Whereas on plastic or metal foils, on polymer substrates, and more generally on very smooth, non porous surfaces, excellent magnetic images are obtainable, the magnetic orientation images obtained on uneven, inhomogeneous fibrous substrates, as well as on porous substrates, are of rather poor quality. Banknote paper falls somewhere in between these extremes of substrates.

On porous or fibrous substrates, the defect most often observed is either an overall reduction of the optical contrast in the magnetic image, or the presence of punctual, small, visible irregularities, characterized by a variation of reflectivity, of color density, or of translucency from one local area to another, which leads to an unpleasant, mottled visual appearance.

WO 2006/061301 A1 discloses a security element having a viewing angle dependent aspect, which can be produced by magnetically orienting platelet-shaped pigment particles in a layer of ink applied over an indicia-carrying background, and subsequently hardening (drying, curing) the ink layer in the oriented state. It was observed that both, the homogeneity and the viewing-angle-dependent optical aspect of the security element, strongly depend on the quality of the substrate onto which the said ink layer is applied. On smooth and non-absorbing substrates, the angle-dependent aspect variation is strong, and large variations of reflectivity and translucency can be observed as a function of the viewing-angle. On fibrous substrates, the angle-dependent aspect variation is poor because the platelet-shaped pigment particles apparently lose their initially imposed magnetic orientation upon drying of the ink.

WO 2003/089250 discloses a method for producing a security document (1) with a security element (2, 3), the security element (2, 3) being produced using a material (M) that is optically changeable by an electric field (E) or magnetic field, the optically changeable material (M) including a plurality of particles (8, 9) that are changeable in their position and/or alignment by means of an electric field (E) or magnetic field, the optically changeable material (M) being produced by enclosing the particles (8, 9) in microcapsules (7) and incorporating them in a binder (6), characterized in that for activating the optically changeable material (M) the microcapsules (7) are brought by a swelling agent into a swollen state in which the particles (8, 9) are supported movably in the microcapsules (7), the optically changeable material (M) being applied to the security document (1) in a nonactivated state.

WO 2009/074284 describes an optically variable security element (12) for securing valuable articles (10), having an optically variable ink layer (40) that includes first, optically variable effect pigments (34) for producing a viewing-angle-dependent visual impression, and that includes second effect pigments (36) that are reversibly alignable by an external magnetic field, the degree of markedness of the viewing-angle-dependent visual impression of the optically variable effect pigments (34) depending on the orientation of the magnetically alignable effect pigments (36) relative to the plane of the ink layer (40).

EP 1 669 213 A1 relates to a security element and to a method of producing the same, the method comprising the steps of (a) providing a substrate having a surface, which surface may contain indicia or other visible features; (b) applying, on top of at least part of the said substrate surface, a coating layer comprising orientable flake pigment particles and a curable, transparent binder; (c) locally orienting said flake pigment particles in said coating layer, such as to give visibility to the underlying substrate surface along at least one specific direction of observation, and to impede visibility to the underlying substrate surface along at least another direction of observation; and (d) curing said coating layer, so as to fix the orientation of the said flake pigment particles; wherein the said flake pigment particles are absorbing in at least part of the visible spectrum.

### Summary of the Invention

Inventors have now found that the said poor quality of the magnetically oriented image on fibrous or porous substrates can be considerably improved by the application of a first coating layer (primer layer) (P) to the fibrous substrate (S), prior to the application of the coating (I) comprising magnetically orientable pigment.

The details of the invention are disclosed hereafter in the description, the drawings and the claims.

The present invention therefore provides a security document or article (D), having
- a substrate (S) selected from woven fibrous substrates, non-woven fibrous substrates, non-fibrous, porous substrates, and non-porous substrates having a textured or uneven surface structure,,
- coated with a first coating layer or first set of coating layers (P), and
- over the first coating layer or first set of coating layers (P), a second coating layer or second set of coating layers (I) comprising at least one type of magnetic or magnetizable particles (F), and a pattern, an image, or indicia being embodied in the second coating layer or second set of coating layers (I) through a homogeneous or locally selective orientation of the particles (F),
wherein the first coating layer or first set of coating layers (P) is/are printed as indicia, lines, raster, grid, logo, geometric patterns, in a way that it selectively impacts the magnetic image in the areas of superposition with the second coating layer or second set of coating layers (I), and which is obtainable by a process comprising the steps of:
a) applying a first coating layer or first set of coating layers (P) to at least part of the surface of a substrate (S);
b) applying, over the first coating layer or first set of coating layers (P), a second coating layer or second set of coating layers (I) comprising at least one type of magnetic or magnetizable particles (F);
c) exposing the second coating layer or second set of coating layers (I) comprising the particles (F), while it is wet, to a magnetic field, thereby allowing the particles (F) to orient in the magnetic field; and
d) hardening the second coating layer or second set of coating layers (I) comprising the particles (F), thereby irreversibly fixing the particles (F) in their respective orientations.

Also, the present invention provides a process for producing the security document or article (D) as defined above, comprising the steps of:
a) applying a first coating layer or first set of coating layers (P) to at least part of the surface of a substrate (S);
b) applying, over the first coating layer or first set of coating layers (P), a second coating layer or second set of coating layers (I) comprising at least one type of magnetic or magnetizable particles (F);
c) exposing the second coating layer or second set of coating layers (I) comprising the particles (F), while it is wet, to a magnetic field, thereby allowing the particles (F) to orient in the magnetic field;
d) hardening the second coating layer or second set of coating layers (I) comprising the particles (F), thereby irreversibly fixing the particles (F) in their respective orientations,
wherein the first coating layer (P) or at least one of the first set of coating layers (P) is printed as indicia, lines, raster, grid, logo, geometric patterns, in a way that it selectively impacts the magnetic image in the areas of superposition with the second coating layer or second set of coating layers (I), and
wherein the substrate (S) is selected from woven fibrous substrates, non-woven fibrous substrates, non-fibrous, porous substrates, and non-porous substrates having a textured or uneven surface structure.

Preferred embodiments of the invention are as defined in the appended dependent claims and/or the following detailed description.

In the present process it is of advantage if said applying a first coating layer (P) includes drying or curing the said first coating layer (P) so as to make it touch-resistant.

In the context of the present invention, the first (primer) coating layer can thus also be a first set of (primer) coating layers (P), for purposes such as increasing the layer thickness or exploiting the opacifying properties of the primer coating. In such case, step (a) of the process is repeated.

More than one second coating layer (I) can further be applied onto the primer-coated substrate, e.g. for obtaining more sophisticated optical effects. In such case, step (b), optionally steps (c), and (d), of the process are repeated, to obtain a second set of coating layers.

The present invention is particularly advantageous if the substrate (S) is a woven fibrous substrate, a non-woven fibrous substrate, non-fibrous, porous substrate, or a non-porous substrate having a textured or uneven surface structure. The substrate may further carry previously applied coatings, such as paper sizing, anti-soiling treatments and offset-printed backgrounds.

The security document or the article (D) can be a bank note, a value document, an identity document, a (such as credit-, access-, identity-) card, a tax excise stamp, a label, a packaging, or a commercial good.

The primer layer may be applied by a large variety of coating processes, such ink- jet printing, offset printing, flexographic printing, gravure printing, screen printing, letterpress printing, decal printing, pad-stamping, and roller-coating; and it can have a thickness ranging from as low as 0.3 µm up to 50 µm or more, depending on the chosen technology. The primer may furthermore be applied in a wet-on-wet process, wherein the subsequent layer is applied without previous drying of the primer layer, or, alternatively the primer layer may be dried prior to the application of the subsequent layer.

It has been found advantageous that the primer coating (P) being dried or cured before the application of the magnetically orientable coating layer; more specifically, the primer coating (P) should be touch-resistant at the moment of applying the magnetically orientable coating layer (I). The preferred curing mechanism is through chemical crosslinking, either through UV-curing, through electron-beam curing, or through oxypolymerizative curing. Simple physical drying through solvent evaporation, solvent absorption into the substrate, or film-forming through coalescence of polymer droplets from an aqueous emulsion, is less efficient, because a so dried layer remains open to re-dissolution under the influence of the subsequently applied coating layer (I). Touch-resistant, in the context of the present disclosure, means that the coating layer will not adhere to a human finger pressed on it.

The first (or primer) coating layer is thus preferably a UV-curing coating composition. Applying a UV coating has the advantage of the technical possibility of instant drying through irradiation with UV light. Instant drying of the first coating (P) allows the second coating (I) to be applied on the same printing machine in a single pass. An alternatively applicable rapid-curing process is electron-beam curing, applicable with electron-beam curing and most other radiation-curing coating compositions.

In case the first coating layer is applied in a previous step, for instance during the substrate production, UV-curing or radiation-curing properties of the coating composition are not necessarily required, as instantaneous drying is not mandatory in such case. An oxypolymerization drying primer can thus be useful as well if the primer coating is performed in a separate process. Physical drying, e.g. through solvent evaporation or through coalescence of polymer droplets from an emulsion, is less preferred as the sole drying mechanism; however, it can be very advantageously used in combination with one of the preceding drying processes in so-called hybrid-curing systems.

Inventors believe that the primer layer principally reduces the paper's ability to take up (absorb), in an either homogeneous or inhomogeneous (localized) manner, part of the ink vehicle. Absorption of a part of the ink vehicle noteworthy results in an effective lowering of the ratio of ink vehicle to pigment in the printed ink film; such lowering of ratio is known to degrade the optical appearance of the magnetic image, as disclosed in WO 2007/131833 A1.

The advantageous drying or curing the primer layer is thought to help blocking the pores of the fibrous or porous substrate, thus preventing absorption, by the substrate, of ink vehicle of the subsequently applied second coating (I), and ensuring therewith that a sufficient amount of liquid is available in the second coating during the subsequent magnetic orientation step, so as to allow the magnetically orientable pigment particles to freely rotate within the ink vehicle and to align with the imposed exterior magnetic field.

A further advantage of the primer layer is to render the printing of the optically variable magnetic ink or the ink containing magnetically orientable pigment particles virtually independent of the chemical and physical properties of the substrate surface. This allows the primer coating to be formulated so as to be compatible with both, the substrate and the ink containing magnetically orientable pigment particles. Such compatibility can be achieved much easier for a primer coating formulation than for the ink formulation comprising magnetically orientable pigment, which, due to its special pigment content, is subject to much more stringent formulation requirements.

In a preferred embodiment, said first coating layer or at least the topmost of said first set of layers (P) has the additional property of promoting the adhesion between the substrate (S) and the said magnetically oriented second coating layer or second set of layers (I).

The first coating (primer) layer (P) may be a colorless, transparent coating or a cholesteric liquid crystal polymer (CLCP) coating. In a preferred embodiment, however, the first coating layer, or at least one of said first set of layers, comprises one or more overt elements selected from the group comprising the soluble dyes and the insoluble pigments. In particular, said pigment may be chosen from the white or colored opaque pigments, the metallic pigments, the iridescent pigments, the optically variable pigments, and the cholesteric liquid crystal polymer (CLCP) pigments.

Said first coating layer or at least one of said first set of layers (I) may further comprise one or more covert element, chosen from the group consisting of the ultraviolet-luminescent compounds, the visible-luminescent compounds, the infrared-luminescent compounds, the up-converting compounds, the infrared-absorbing compounds, the magnetic compounds, and the forensic taggants.

An overt element, in the context of the present description, is a material which can be admixed to, or which is otherwise part of a coating composition, and which exhibits at least one visibly distinctive property, such as color, color-shift or iridescence. Overt elements can be visually authenticated.

A covert element, in the context of the present description, is a material which can be admixed to, or which is otherwise part of a coating composition, and which exhibits at least one non-visibly distinctive property, such as luminescence, magnetism or IR-absorption. Covert elements need particular equipment for their authentication.

In a particular embodiment, said first coating layer or at least one of said first set of layers comprises a cholesteric liquid crystal polymer (CLCP) material, exhibiting viewing-angle dependent color and reflecting a circularly polarized light component within a determined wavelength range.

Said first coating layer or at least one of said first set of layers (P) may further carry information, such as a serial number or personalization information, being inscribed by a method of variable-information-printing, preferably by laser marking.

The magnetic or magnetizable particles (F) of the second coating layer or set of second layers (I) are preferably embodied by a magnetic flake pigment, more preferably by optically reflective magnetic pigment flakes.

The magnetic or magnetizable particles (F) of the second coating layer or set of second layers (I) can also be advantageously embodied by an optically variable magnetic pigment, preferably by a thin-film interference pigment comprising either an {absorber layer / dielectric layer / reflecting magnetic layer}, or an {absorber layer / dielectric layer / reflector layer plus a magnetic layer} sequence. In the latter sequence, the magnetic functionality is separated from the reflector functionality, and embodied as an additional layer, which may either be located adjacent to the reflector layer, or separated from the reflector layer by one or more additional layers.

Said second coating layer, or at least one of said second set of layers (I), may further comprise one or more covert elements, chosen from the group consisting of the ultraviolet-luminescent compounds, the visible-luminescent compounds, the infrared-luminescent compounds, the up-converting compounds, the infrared- absorbing compounds, the magnetic compounds, and the forensic taggants.

In a particularly preferred embodiment of the method, said second coating layer (I) comprising said at least one type of magnetic or magnetizable particles (F), is exposed, while it is wet, to the magnetic field of an indicia-engraved, permanent magnetic plate, such as disclosed in WO 2005/002866 A1 or in the co-pending application WO 2008/046702 A1, and hardened during or after said exposition. This allows achieving a line width (r) of the obtained magnetic orientation pattern, image or indicia which is lower than 3 mm, preferably lower than 2 mm, most preferably lower than 1 mm.

Said first coating layer, or at least one of said first set of layers (P), is printed in the form of indicia, lines, raster, grid, logo, geometric patterns, in a way that it selectively impacts the magnetic image in the areas of superposition with the second coating layer or second set of layers (I).

### Detailed Description of the Invention

The present invention comprises a process for producing a security document or article (D) as defined above, comprising the steps of:
a) applying a first coating layer or first set of coating layers (P) to at least part of the surface of a substrate (S);
b) applying, over the first coating layer or first set of coating layers (P), a second coating layer or second set of coating layers (I) comprising at least one type of magnetic or magnetizable particles (F);
c) exposing the second coating layer or second set of coating layers (I) comprising the particles (F), while it is wet, to a magnetic field, thereby allowing the particles (F) to orient in the magnetic field;
d) hardening the second coating layer or second set of coating layers (I) comprising the particles (F), thereby irreversibly fixing the particles (F) in their respective orientations,
wherein the first coating layer (P) or at least one of the first set of coating layers (P) is printed as indicia, lines, raster, grid, logo, geometric patterns, in a way that it selectively impacts the magnetic image in the areas of superposition with the second coating layer or second set of coating layers (I), and
wherein the substrate (S) is selected from woven fibrous substrates, non-woven fibrous substrates, non-fibrous, porous substrates, and non-porous substrates having a textured or uneven surface structure.

Said pattern, image, or indicia may be everything which can be produced through the orientation, in a homogeneous or in a locally selective way, of anisotropic particles, i.e. needles or flakes, comprised in a coating. In homogeneous orientation, all particles of a determined surface area adopt a same, common direction, such as disclosed in WO 2006/061301 A1, whereas in locally selective orientation, the particles adopt locally varying direction, so as to represent a pattern, an image, a logo, or still other types of indicia.

The invention further comprises a security document or an article (D), obtainable by the present process, having
- a substrate (S) selected from woven fibrous substrates, non-woven fibrous substrates, non-fibrous, porous substrates, and non-porous substrates having a textured or uneven surface structure,
- coated with a first coating layer or first set of coating layers (P), and
- over the first coating layer or first set of coating layers (P), a second coating layer or second set of coating layers (I) comprising at least one type of magnetic or magnetizable particles (F), and a pattern, an image, or indicia being embodied in the second coating layer or second set of coating layers (I) through a homogeneous or locally selective orientation of the particles (F),
wherein the first coating layer or first set of coating layers (P) is/are printed as indicia, lines, raster, grid, logo, geometric patterns, in a way that it selectively impacts the magnetic image in the areas of superposition with the second coating layer or second set of coating layers (I).

The substrate of the security document or article (D) is selected from woven fibrous substrates, non-woven fibrous substrates, non-fibrous, porous substrates (such as a plastic substrate having a porous surface), and non-porous substrates having a textured or uneven surface structure. The substrate may be opaque, transparent or translucent. It can further be colorless or colored. The substrate may be uncoated, or pre-coated with, for example, sizing agents or anti-soiling treatments, it may further be blank or carry printings, such as an offset background.

The process according to the present invention is advantageously used for the production of security documents or articles (D), such as bank notes, value documents, identity documents, cards, tax excise stamps, labels and packaging, as well as for the marking of commercial goods against counterfeiting and diversion (product security applications).

The first, or primer coating layer, which can also be a first set of layers (P), has a thickness in the range of 0.3-50 µm. The crucial layer considered in the context of the present invention is the topmost of said set of layers (P) in case the document carries a multiple coating, comprising e.g. paper treatments or background printings.

The said first coating layer (P) may be applied by any printing process known in the art, in particular a process chosen from the group consisting of ink-jet printing, offset printing, flexographic printing, gravure printing, screen printing, letterpress printing, decal printing, pad-stamping, and roller-coating; however it is most preferably applied by one of the flexographic, gravure or screen-printing processes. Said first coating layer (P) is printed as lines, raster, grid, logo, geometric patterns, in a way that it selectively impacts the magnetic image in the areas of superposition with the second coating layer (I).

The coating layer (P) is most preferably a radiation-curable coating, such as a UV or electron beam coating composition, e.g. a UV-drying screen printing ink, or a UV drying ink-jet, offset, flexography, gravure ink or roller coating ink. Radiation curing noteworthy results in a rapid (instant) drying, and therefore allows for high production speeds on the printing press. When the coating layer is applied in a previous step of the production, and when therefore an instantaneous drying is not mandatory, it can be also a solvent-based or a water-based coating, drying by evaporation or penetration of its constitutive solvents, or by any other drying process, such as oxypolymerisation or chemical crosslinking.

Although wet-on-wet processes are possible, wherein the second coating is applied onto the primer coating without previous drying the latter, said primer (P) is preferably dried or cured prior to the application of the magnetically orientable coating (I). Such drying or curing is helpful to obtain the best effect out of the present invention. The primer coating layer should be cured at least to the point where it is touch-resistant, i.e. where it does no longer show any set-off and can touch the printing equipment, for the application of the second layer, without being damaged or soiling the printing equipment. Said drying may be achieved, according to the chemical nature of the primer coating, through UV-radiation, electron-beam radiation, heating, or still other drying or curing mechanisms which lead to a hardening of the coating.

Primer coatings (P) based on other chemistries, such as water-based emulsion coating compositions, solvent-based thermoplastic or thermosetting coating compositions, air-drying coating compositions, hybrid compositions including water-based/UV curing and solvent-based/UV curing components may be used as well.

The primer coating is thus chosen from the group consisting of the UV-curing coatings, the solvent-based coatings, the water-based coatings including but not limited to the emulsion coatings, the oxidatively drying coatings, the water-based/UV drying hybrid coatings and the solvent-based/UV drying hybrid coatings.

In a particular embodiment, said first coating layer or at least one of said first set of layers comprises a cholesteric liquid crystal polymer (CLCP) material, exhibiting viewing-angle dependent color and reflecting a circularly polarized light component within a determined wavelength range. Such materials, disclosed e.g. in US 5,798,147 (Beck et al.) and US 6,899,824 (Meyer et al.), can be applied in the form of a precursor liquid crystal coating, which, when subject to determined external conditions (temperature), develops a characteristically colored cholesteric texture. The cholesteric texture is then "frozen" through the photopolymerization of the precursor material.

In another embodiment, the topmost primer layer (P) is a colorless, transparent coating. In another preferred embodiment, the primer coating comprises a soluble dye and/or an insoluble pigment. A colored dye or pigment can be chosen so as to reinforce the optical effect of the optically variable magnetic ink and the magnetic image overprinted on top of the primer. Preferably said pigment is chosen from the white or colored opaque pigments, the metallic pigments, the iridescent pigments, the optically variable pigments, and the mixtures thereof.

An optical effect pigment, such as a color shifting, an iridescent, or a metallic pigment, can provide additional security to the document whilst enriching the overall aspect of the magnetic image.

In a particularly preferred embodiment, said primer (P) comprises one or more transparent or colored cholesteric liquid crystal polymer (CLCP) pigments, exhibiting viewing-angle dependent color and reflecting circularly polarized light of a determined sense within a determined wavelength range.

Cholesteric liquid crystal polymers have a molecular order in the form of helically arranged molecular stacks. This order is at the origin of a periodic spatial modulation of the material's refractive index, which in tum results in a selective transmission / reflection of determined wavelengths and polarization senses of light. The particular situation of the helical molecular arrangement in CLCPs causes the reflected light to be circular polarized, left-handed or right-handed, depending on the sense of rotation of the molecular helical stack. The presence of circular polarization as an additional hidden feature is a further security element.

The preferred CLCP pigments are flakes of the type described in EP 1 876 216 A1, EP 1 213 338 B1; EP 0 685 749 B1; DE 199 22 158 A1; EP 0 601 483 A1; DE 44 18 490 A1; EP 0 887 398 B1, and WO 2006/063926, as well as in US 5,211,877, US 5,362,315 and US 6,423,246. The pigment particles have a thickness of the order of 1-10 µm and a flake size of the order of 10-100 µm, and are obtained by comminution of a corresponding liquid-crystal polymer precursor film.

The primer coating (P) may further comprise covert security elements, chosen from ultraviolet-luminescent compounds, visible-luminescent compounds, infrared-luminescent compounds, up-converting compounds, infrared-absorbing compounds, magnetic pigments, and forensic taggants.

Luminescent dyes or pigments, as well as infrared-absorbing compound can provide the document with additional covert and machine-readable security markings, providing for machine-authenticate-ability of the security document according to established technology. A magnetic pigment in the primer layer can additionally provide for cooperative effects with the oriented optically variable magnetic pigment in the second layer. A forensic security marker, such as disclosed in EP 0 927 750 B1, can provide for trace-ability of an ink marked therewith, and of the correspondingly printed documents.

Said first coating layer (P) may further carry information, such as a serial number or personalization information, which may be applied by a method of variable-information-printing, such as laser marking.

Said primer (P) may have the additional property or function to promote the adhesion between the substrate (S) and the magnetically oriented coating layer (I). Such may be noteworthy required in the case of surface-treated paper, having e.g. an anti-soiling coating, such as is frequently used for banknote printing. Anti-soiling coated papers are difficult to imprint with standard ink formulations. On the other hand, changing a functional ink formula, such as an optically variable magnetic ink, so as to additionally exhibit improved adhesion properties is a difficult task. Providing a primer coating composition having adhesion-promoting functionality is much easier to achieve and is thus a preferred choice in case of adhesion problems.

Said magnetic or magnetizable particles (F) in said second coating layer or second set of layers (I) are preferably embodied by magnetic pigment flakes, such as iron flakes, most preferably either by optically reflective magnetic pigment flakes, as disclosed in US 6,818,299 (Phillips et al.), or by optically variable magnetic pigment, such as disclosed in US 4,838,648; in EP 686,675 B1; in WO 02/73250 A2 and in WO 03/00801 A2.

An exemplary embodiment of optically reflective magnetic pigment flakes is a thin-film pigment comprising a reflector layer/magnetic layer/reflector thin-layer sequence, e.g. realized in MgF₂/Al/Ni/Al/MgF₂, wherein the reflector layers are embodied by aluminum, and the magnetic layer is embodied by nickel.

The magnetic or magnetizable particles (F) in said second coating layer or second set of layers (I) are most preferably embodied by optically variable magnetic pigment.

An exemplary embodiment of optically variable magnetic pigment is a thin-film interference pigment comprising either an absorber layer I dielectric layer I reflecting magnetic layer, or an absorber layer I dielectric layer I reflector layer plus magnetic layer sequence. Such pigment is based on a Fabry-Pérot resonator structure, wherein the wavelengths of reflected light are determined by the optical thickness of the dielectric layer. Pigments having separate magnetic and optical reflector layers are advantageously used, because they allow to freely combine magnetic and optical reflecting properties, as is disclosed in EP 1 266 380 B1.

The orientation of the pigment particles (F) in the wet printed ink or coating composition (I) is imposed by the external applied magnetic field. A minimum thickness of the ink film layer (I) on the substrate is required to allow for rotational freedom of the magnetic pigment particles (e.g. flakes, F) in the ink medium, such that the pigment particles (F) can freely align with the applied magnetic field. The second coating is therefore applied in a typical film thickness of 10-30 µm.

The process of the present invention is particularly advantageous in the case of the magnetic orientation transfer of a fine line pattern or of high-resolution indicia, such as disclosed in WO 2005/002866 A1 and in the co-pending application WO 2008/046702 A1. It has been found that an excellent quality of the magnetically transferred image is required if this latter contains fine line details, and that, in order to correctly transfer fine line details onto a fibrous substrate such as banknote paper, a primer coating according to the disclosure of the present invention is essential and strongly improves the optical appearance of the magnetically oriented security element.

A fine line detail in the context of the present invention is to be understood as having a line width (r) lower than 3 mm. Using the devices disclosed in WO 2005/002866 A1 and in WO 2008/046702 A1, line widths lower than 2 mm, and even lower than 1 mm can be easily transferred as a magnetic orientation pattern. Fig. 2 illustrates the line width (r) of a pattern obtained by magnetic transfer into the second coating (I), and how it is linked to the nature of the magnetic field lines of the magnetic orientation plate (M).

In the present invention, said first coating layer (P) is printed as lines, raster, grid, logo, geometric patterns, in a way that it selectively impacts the magnetic image in the areas of superposition with the second coating layer (I). Particularly preferred is further a document or article (D) comprising a fine-line magnetic image, i.e. wherein the said indicia have a line width (r) lower than 3mm, preferably lower than 2mm, most preferably lower than 1mm; such indicia can be produced using the orientation devices disclosed in WO 2005/002866 A1 or in WO 2008/046702 A1.

The invention is now further explained with respect to the drawings and exemplary embodiments.

### Brief Description of the Drawings

- **Fig. 1**: schematically illustrates the security element of the present invention: S is the fibrous or porous substrate; P is the first coating (primer coating), I is the second coating comprising at least one type of magnetic or magnetizable particles (F), wherein indicia are embodied through a selective orientation of the said magnetic or magnetizable particles (F).
- **Fig. 2**: illustrates the dependency of the line width (r) of a pattern, obtained by magnetic orientation of particles in a coating (I), of the magnetic field used to orient the particles. Fine-line patterns require abrupt reversals of the magnetic field.
- **Fig. 3**: illustrates the effect of the applied primer layer (P) on the formation of magnetic orientation images on a "difficult" substrate (absorbing offset paper):
a) optically variable magnetic ink (I) directly printed onto the substrate (S), followed by magnetic orientation of the pigment and hardening of the ink: no image is visible;
b) optically variable magnetic ink (I) printed onto a primer layer (P) of the present invention, otherwise same conditions as in (a): The magnetic orientation image appears clear and neat.
c) optically variable magnetic ink (I) printed half on a primer layer (P), half on the substrate (S), otherwise same conditions as in (a): The magnetic orientation image appears clear and neat in the primer-coated part (left), but not at all in the uncoated part (right).

### Examples

### Ink formulas

Inks for the first (primer) coating (P) are made as known to the skilled person. A first example of a UV-curing primer formula for the application by the flexography process is as follows:

| | |
|---|---|
| Epoxyacrylate oligomer | 49% |
| Trimethylolpropane triacrylate monomer (TMPTA) | 20% |
| Tripropyleneglycol diacrylate monomer (TPGDA) | 20% |
| Genorad 16 (Rahn) | 1% |
| Aerosil 200 (Degussa-Huels) | 2% |
| Irgacure 500 (Ciba) | 6% |
| Genocure EPD (Rahn) | 2% |

A second, alternative UV-drying primer comprising a luminescent marker for the application by silkscreen printing is formulated as follows:

| | |
|---|---|
| Epoxyacrylate oligomer | 47% |
| Trimethylolpropane triacrylate monomer (TMPTA) | 20% |
| Tripropyleneglycol diacrylate monomer (TPGDA) | 20% |
| Luminnescent pigment (Cartax CXDP, supplied by Clariant) | 3% |
| Genorad 16 (Rahn) | 1% |
| Aerosil 200 (Degussa-Huels) | 1% |
| Irgacure 500 (Ciba) | 6% |
| Genocure EPD (Rahn) | 2% |

A third example consists in a 2 layers primer. The substrate is first printed with an oxidative drying process magenta sheet-fed offset ink. Once this first layer is dried, a UV-drying screen-printing primer, comprising a LCP flake pigment, is applied on the offset layer. The formulation of the silkscreen primer is the following:

| | |
|---|---|
| Epoxyacrylate oligomer | 43% |
| Trimethylolpropane triacrylate monomer (TMPTA) | 18% |
| Tripropyleneglycol diacrylate monomer (TPGDA) | 18% |
| Helicone HC Maple S (LCP Technologies) | 10% |
| Genorad 16 (Rahn) | 1% |
| Aerosil 200 (Degussa-Huels) | 2% |
| Irgacure 500 (Ciba) | 6% |
| Genocure EPD (Rahn) | 2% |

The second coating composition (I), comprising magnetic optically variable pigment, is formulated as disclosed in WO 2007/131833 A1. An example of a UV-drying silk-screen ink formula is as follows:

| | |
|---|---|
| Epoxyacrylate oligomer | 40% |
| Trimethylolpropane triacrylate monomer (TMPTA) | 10% |
| Tripropyleneglycol diacrylate monomer (TPGDA) | 10% |
| Genorad 16 (Rahn) | 1% |
| Aerosil 200 (Degussa-Huels) | 1% |
| Irgacure 500 (CIBA) | 6% |
| Genocure EPD (Rahn) | 2% |
| Magnetic optically variable pigment (5 layers)* | 20% |
| Dowanol PMA | 10% |

| | |
|---|---|
| Viscosity (mPa.s, Brookfield) 800 * supplied by FLEX Products, Inc., Santa Rosa, CA | |

### Printing and magnetic orientation (Reference, not according to the Invention)

A first sheet of standard offset paper was used as such. A second sheet of standard offset paper was silk-screen imprinted as a solid surface with 24 µm of the first primer composition given here above, and the printed composition was UV-cured.

Both papers were silk-screen imprinted with a solid patch of the second coating composition (I) given here above, in a thickness of 30 µm. The imprinted substrates were briefly placed on an indicia-carrying magnetic plate such as disclosed in WO 2008/046702 A1 and in WO 2005/002866 A1, and the oriented coatings were UV-cured.

Fig. 3 shows the results obtained under otherwise same conditions: On the paper which was not primer-coated, the magnetic orientation image is not visible (Fig. 3a); whereas on the primer-coated paper, the magnetic orientation image is clear and neat (Fig. 3b). If the indicia-carrying magnetic plate is made to overlap coated and non-coated areas of the second substrate during the image-forming step, then the image is formed only clear and neat where the primer (P) coating is present (Fig. 3c).

## Claims

1. A security document or article (D), having
- a substrate (S) selected from woven fibrous substrates, non-woven fibrous substrates, non-fibrous, porous substrates, and non-porous substrates having a textured or uneven surface structure,,
- coated with a first coating layer or first set of coating layers (P), and
- over the first coating layer or first set of coating layers (P), a second coating layer or second set of coating layers (I) comprising at least one type of magnetic or magnetizable particles (F), and a pattern, an image, or indicia being embodied in the second coating layer or second set of coating layers (I) through a homogeneous or locally selective orientation of the particles (F),
wherein the first coating layer or first set of coating layers (P) is/are printed as indicia, lines, raster, grid, logo, geometric patterns, in a way that it selectively impacts the magnetic image in the areas of superposition with the second coating layer or second set of coating layers (I), and
which is obtainable by a process comprising the steps of:
a) applying a first coating layer or first set of coating layers (P) to at least part of the surface of a substrate (S);
b) applying, over the first coating layer or first set of coating layers (P), a second coating layer or second set of coating layers (I) comprising at least one type of magnetic or magnetizable particles (F);
c) exposing the second coating layer or second set of coating layers (I) comprising the particles (F), while it is wet, to a magnetic field, thereby allowing the particles (F) to orient in the magnetic field; and
d) hardening the second coating layer or second set of coating layers (I) comprising the particles (F), thereby irreversibly fixing the particles (F) in their respective orientations.

2. The security document or article of claim 1, wherein the first coating layer or first set of coating layers (P) has a thickness of 0.3-50 µm.

3. The security document or article f claim 1 or 2, wherein the first coating layer (P) or at least the topmost of the first set of coating layers (P) is applied by a process chosen from ink-jet printing, offset printing, flexographic printing, gravure printing, screen printing, letterpress printing, decal printing, pad-stamping, and roller-coating.

4. The security document or article of any of claims 1-3,
wherein the first coating layer (P) or at least the topmost of the first set of coating layers (P) is chosen from UV-curing coating compositions, electron-beam-curing coating compositions, solvent-based coating compositions, water-based coating compositions, oxypolymerization drying coating compositions, and hybrid-curing coating compositions including water-based/UV curing and solvent-based/UV curing coatings.

5. The security document or article of any of claims 1-4,
wherein the first coating layer (P) or at least the topmost of the first set of coating layers (P) is a colorless transparent coating.

6. The security document or article of any of claims 1-5,
wherein the first coating layer (P) or at least one of the first set of coating layers (P) comprises a cholesteric liquid crystal polymer (CLCP) material, exhibiting viewing-angle dependent color and reflecting a circularly polarized light component within a determined wavelength range.

7. The security document or article of any of claims 1-6,
wherein the first coating (P) or at least one of the first set of coating layers (P) comprises one or more overt elements selected from soluble dyes and insoluble pigments.

8. The security document or article of claim 7, wherein the pigment is chosen from white or colored opaque pigments, metallic pigments, iridescent pigments, optically variable pigments, and cholesteric liquid crystal polymer (CLCP) pigments.

9. The security document or article of any of claims 1-8,
wherein the first coating (P) or at least one of the first set of coating layers (P) comprises one or more covert elements, chosen from ultraviolet-luminescent compounds, visible-luminescent compounds, infrared-luminescent compounds, up-converting luminescent compounds, infrared-absorbing compounds, magnetic compounds, and forensic taggants.

10. The security document or article of any of claims 1-9
wherein the first coating (P) or at least one of the first set of coating layers (P) carries information, such as a serial number or personalization information, being inscribed by a method of variable-information-printing, preferably by laser marking.

11. The security document or article of any of claims 1-10,
wherein the first coating layer (P) or at least the topmost of the first set of coating layers (P) has the additional property of promoting the adhesion between the substrate (S) and the magnetically oriented layer second coating layer or second set of coating layers (I).

12. The security document or article of any of claims 1-11,
wherein the particles (F) in the second coating layer or second set of coating layers (I) are embodied by magnetic pigment flakes, preferably by optically reflective magnetic pigment flakes.

13. The security document or article of any of claims 1-11,
wherein the particles (F) in the second coating layer or second set of coating layers (I) (I) are embodied by optically variable magnetic pigment, preferably by thin-film interference pigment comprising either an absorber layer/dielectric layer/reflecting magnetic layer, or an absorber layer/dielectric layer/reflector layer plus a magnetic layer sequence.

14. The security document or article of any of claims 1-13,
wherein the second coating layer (I) or at least one of the second set of coating layers (I) comprises one or more covert elements, chosen from ultraviolet-luminescent compounds, visible-luminescent compounds, infrared-luminescent compounds, up- converting compounds, infrared-absorbing compounds, magnetic compounds, and forensic taggants.

15. The security document or article of any of claims 1-14,
wherein the line width (r) of the magnetic orientation pattern, image or indicia is < 3 mm, preferably < 2 mm, most preferably < 1 mm.

16. The security document or article of any of claims 1-15, which is selected from bank notes, value documents, identity documents, cards, tax excise stamps, labels, packaging, and commercial goods.

17. A process for producing the security document or article of any of claims 1-16, comprising the steps of:
a) applying a first coating layer or first set of coating layers (P) to at least part of the surface of a substrate (S);
b) applying, over the first coating layer or first set of coating layers (P), a second coating layer or second set of coating layers (I) comprising at least one type of magnetic or magnetizable particles (F);
c) exposing the second coating layer or second set of coating layers (I) comprising the particles (F), while it is wet, to a magnetic field, thereby allowing the particles (F) to orient in the magnetic field;
d) hardening the second coating layer or second set of coating layers (I) comprising the particles (F), thereby irreversibly fixing the particles (F) in their respective orientations, and
wherein the first coating layer (P) or at least one of the first set of coating layers (P) is printed as indicia, lines, raster, grid, logo, geometric patterns, in a way that it selectively impacts the magnetic image in the areas of superposition with the second coating layer or second set of coating layers (I),
wherein the substrate (S) is selected from woven fibrous substrates, non-woven fibrous substrates, non-fibrous, porous substrates, and non-porous substrates having a textured or uneven surface structure.

18. The process of claim 17, wherein step (a) includes drying or curing the first coating layer or first set of coating layers (P) so as to make it touch-resistant.

19. The process of claim 18, wherein the drying or curing is performed by a process selected from UV-curing, electron-beam curing, oxypolymerization drying, physical drying, and combinations thereof.

20. The process of any of claims 17-19, wherein the first coating layer (P) or at least the topmost of the first set of coating layers (P) is applied by a printing process selected from ink-jet printing, offset printing, flexographic printing, gravure printing, screen printing, letterpress printing, decal printing, pad-stamping, and roller-coating.

21. The process of any of claims 17-20, wherein information, such as a serial number or personalization information, is inscribed in the first coating layer (P) or at least one of the first set of coating layers (P) by a method of variable-information-printing, preferably by laser marking.

22. The process of any of claims 17-21, wherein the particles (F) in the second coating layer or second set of coating layers (I) are embodied by magnetic pigment flakes, preferably by optically reflective magnetic pigment flakes.

23. The process of any of claims 17-21, wherein the particles (F) in the second coating layer or second set of coating layers (I) are embodied by optically variable magnetic pigment, preferably by thin-film interference pigment comprising either an absorber layer/dielectric layer/reflecting magnetic layer, or an absorber layer/dielectric layer/reflector layer plus a magnetic layer sequence.

24. The process of any of claims 17-23, wherein the first coating layer or first set of coating layers is/are applied over a coating comprising a cholesteric liquid crystal polymer (CLCP) material.

25. The process of any of claims 17-24, wherein the second coating layer or second set of coating layers (I) comprising the particles (F) is/are exposed while it is wet to the magnetic field of an indicia-engraved, permanent magnetic plate.

## Patentansprüche

1. Ein Sicherheitsdokument oder -artikel (D), umfassend
- ein Substrat (S), ausgewählt aus gewebten Fasersubstraten, ungewebten Fasersubstraten, unfaserigen porösen Substraten und unporösen Substraten mit einer texturierten oder unebenen Oberflächenstruktur,
- beschichtet mit einer ersten Überzugsschicht oder einem ersten Satz von Überzugsschichten (P), und
- über der ersten Überzugsschicht oder dem ersten Satz von Überzugsschichten (P), eine zweite Überzugsschicht oder einen zweiten Satz von Überzugsschichten (I), die/der mindestens eine Art von magnetischen oder magnetisierbaren Partikeln (F) umfasst, und ein Muster, ein Bild, oder Indizien, die in der zweiten Überzugsschicht oder dem zweiten Satz von Überzugsschichten (I) durch eine homogene oder lokal selektive Orientierung der Partikel (F) gebildet sind,
wobei die erste Überzugsschicht oder der erste Satz von Überzugsschichten (P) als Indizien, Linien, Raster, Gitter, Logo und geometrische Muster derart gedruckt wird, dass sie/er das magnetische Bild in den Überlagerungsbereichen mit der zweiten Überzugsschicht oder dem zweiten Satz von Überzugsschichten (I) selektiv beeinflussen, und
welches durch ein Verfahren erhalten wird, das die folgenden Schritte umfasst:
a) Aufbringen einer ersten Überzugsschicht oder eines ersten Satzes von Überzugsschichten (P) auf mindestens einen Teil der Oberfläche eines Substrats (S);
b) Aufbringen einer zweiten Überzugsschicht oder eines zweiten Satzes von Überzugsschichten (I), die/der mindestens eine Art von magnetischen oder magnetisierbaren Partikeln (F) umfasst, über die erste Überzugsschicht oder den ersten Satz von Überzugsschichten (P);
c) Aussetzen der zweiten Überzugsschicht oder des zweiten Satzes von Überzugsschichten (I), die/der die Partikeln (F) umfassen, während sie/er nass ist, gegenüber einem Magnetfeld, wodurch sich die Partikeln (F) im Magnetfeld orientieren können; und
d) Härten der zweiten Überzugsschicht oder des zweiten Satzes von Überzugsschichten (I), die/der die Partikeln (F) umfassen, wodurch die Partikeln (F) in ihren jeweiligen Orientierungen irreversibel fixiert werden.

2. Das Sicherheitsdokument oder -artikel nach Anspruch 1, wobei die erste Überzugsschicht oder der erste Satz von Überzugsschichten (P) eine Dicke von 0,3 bis 50 µm aufweist.

3. Das Sicherheitsdokument oder -artikel nach Anspruch 1 oder 2, wobei die erste Überzugsschicht (P) oder mindestens die oberste Schicht des ersten Satzes von Überzugsschichten (P) durch ein Verfahren aufgebracht wird, das aus dem Tintenstrahldruck, Offsetdruck, Flexodruck, Tiefdruck, Siebdruck, Buchdruck, Abziehbilddruck, Tampondruck und Rollenbeschichten ausgewählt wird.

4. Das Sicherheitsdokument oder -artikle nach einem der Ansprüche 1 bis 3, wobei die erste Überzugsschicht (P) oder mindestens die oberste Schicht des ersten Satzes von Überzugsschichten (P) aus UV-härtenden Beschichtungszusammensetzungen, durch Elektronenstrahl härtenden Beschichtungszusammensetzungen, Beschichtungszusammensetzungen auf Lösungsmittelbasis, Beschichtungszusammensetzungen auf Wasserbasis, durch Oxypolymerisation trocknenden Beschichtungszusammensetzungen und hybridisiert härtenden Beschichtungszusammensetzungen, einschließlich auf Wasser basierende/UV-härtende und auf Lösungsmittel basierende/UV-härtende Beschichtungen, ausgewählt wird.

5. Das Sicherheitsdokument oder -artikel nach einem der Ansprüche 1 bis 4, wobei die erste Überzugsschicht (P) oder mindestens die oberste Schicht des ersten Satzes von Überzugsschichten (P) eine farblose transparente Beschichtung ist.

6. Das Sicherheitsdokument oder -artikel nach einem der Ansprüche 1 bis 5, wobei die erste Überzugsschicht (P) oder mindestens eine des ersten Satzes von Überzugsschichten (P) ein cholesterisches Flüssigkristallpolymeren(CFKP)-Material umfasst, das eine winkelabhängige Farbe aufweist und eine kreisförmig polarisierte Lichtkomponente innerhalb eines bestimmten Wellenlängenbereichs reflektiert.

7. Das Sicherheitsdokument oder -artikel nach einem der Ansprüche 1 bis 6, wobei die erste Überzugsschicht (P) oder mindestens eine des ersten Satzes von Überzugsschichten (P) ein oder mehrere offene Elemente umfasst, die aus löslichen Farbstoffen und unlöslichen Pigmenten ausgewählt sind.

8. Das Sicherheitsdokument oder -artikel nach Anspruch 7, wobei das Pigment ausweißen oder farbigen, undurchsichtigen Pigmenten, Metallpigmenten, irisierenden Pigmenten, optisch variablen Pigmenten und cholesterischen Flüssigkristallpolymer (CFKP)-Pigmenten ausgewählt ist.

9. Das Sicherheitsdokument oder -artikel nach einem der Ansprüche 1 bis 8, wobei die erste Überzugsschicht (P) oder mindestens eine des ersten Satzes von Überzugsschichten (P) ein oder mehrere verdeckte Elemente umfasst, die aus Ultraviolett-Lumineszenzverbindungen, sichtbaren Lumineszenzverbindungen, Infrarot-Lumineszenzverbindungen, aufwärts konvertierenden Lumineszenzverbindungen, Infrarot absorbierenden Verbindungen, magnetischen Verbindungen und forensischen Taggants ausgewählt sind.

10. Das Sicherheitsdokument oder -artikel nach einem der Ansprüche 1 bis 9, wobei die erste Überzugsschicht (P) oder mindestens eine des ersten Satzes von Überzugsschichten (P) Informationen wie eine Seriennummer oder Personalisierungsinformationen trägt, die durch ein Verfahren zum Drucken von variablen Informationen, vorzugsweise durch Lasermarkierung, eingeschrieben sind.

11. Das Sicherheitsdokument oder -artikel nach einem der Ansprüche 1 bis 10, wobei die erste Überzugsschicht (P) oder mindestens die oberste Schicht des ersten Satzes von Überzugsschichten (P) die zusätzliche Eigenschaft hat, die Haftung zwischen dem Substrat (S) und der magnetisch orientierten zweiten Überzugsschicht oder dem zweiten Satz von Überzugsschichten (I) vermittelt.

12. Das Sicherheitsdokument oder -artikel nach einem der Ansprüche 1 bis 11, wobei die Partikeln (F) in der zweiten Überzugsschicht oder dem zweiten Satz von Überzugsschichten (I) von magnetischen Pigmentflocken, vorzugsweise von optisch reflektierenden magnetischen Pigmentflocken, gebildet sind.

13. Das Sicherheitsdokument oder -artikel nach einem der Ansprüche 1 bis 11, wobei die Partikeln (F) in der zweiten Überzugsschicht oder dem zweiten Satz von Überzugsschichten (I) von einem optisch variablen magnetischen Pigment, vorzugsweise von einem Dünnfilminterferenz-Pigment, gebildet werden, das entweder eine Absorberschicht/dielektrische Schicht/reflektierende magnetische Schicht oder eine Absorberschicht/dielektrische Schicht/Reflektorschicht plus eine magnetische Schichtenfolge umfasst.

14. Das Sicherheitsdokument oder -artikel nach einem der Ansprüche 1 bis 13, wobei die zweite Überzugsschicht (I) oder mindestens eine des zweiten Satzes von Überzugsschichten (I) ein oder mehrere verdeckte Elemente umfasst, die aus Ultraviolett-Lumineszenzverbindungen, sichtbaren Lumineszenzverbindungen, Infrarot-Lumineszenzverbindungen, aufwärts konvertierenden Lumineszenzverbindungen, Infrarot absorbierenden Verbindungen, magnetischen Verbindungen und forensischen Taggants ausgewählt sind.

15. Das Sicherheitsdokument oder -artikel nach einem der Ansprüche 1 bis 14, wobei die Linienbreite (r) des magnetischen Orientierungsmusters, Bildes oder der Indizien <3 mm, vorzugsweise <2 mm, am meisten bevorzugt <1 mm ist.

16. Das Sicherheitsdokument oder -artikel nach einem der Ansprüche 1 bis 15, ausgewählt aus Banknoten, Wertdokumenten, Ausweisdokumenten, Karten, Steuerbelastungsmarken, Etiketten, Verpackungen und Handelswaren.

17. Ein Verfahren zur Herstellung des Sicherheitsdokuments oder -artikels nach einem der Ansprüche 1 bis 16, das die folgenden Schritte umfasst:
a) Aufbringen einer ersten Überzugsschicht oder eines ersten Satzes von Überzugsschichten (P) auf mindestens einen Teil der Oberfläche eines Substrats (S);
b) Aufbringen einer zweiten Überzugsschicht oder eines zweiten Satzes von Überzugsschichten (I), die/der mindestens eine Art von magnetischen oder magnetisierbaren Partikeln (F) umfasst, über die erste Überzugsschicht oder den ersten Satz von Überzugsschichten (P);
c) Aussetzen der zweiten Überzugsschicht oder des zweiten Satzes von Überzugsschichten (I), die/der die Partikeln (F) umfassen, gegenüber einem Magnetfeld, während sie/er nass ist, wodurch sich die Partikeln (F) im Magnetfeld orientieren können;
d) Härten der zweiten Überzugsschicht oder des zweiten Satzes von Überzugsschichten (I), die/der die Partikeln (F) umfassen, wodurch die Partikeln (F) in ihren jeweiligen Orientierungen irreversibel fixiert werden, und
wobei die erste Überzugsschicht (P) oder mindestens eine des ersten Satzes von Überzugsschichten (P) als Indizien, Linien, Raster, Gitter, Logo und geometrische Muster derart gedruckt wird, dass sie/er das magnetische Bild in den Überlagerungsbereichen mit der zweiten Überzugsschicht oder dem zweiten Satz von Überzugsschichten (I) selektiv beeinflussen,
wobei das Substrat (S) aus gewebten Fasersubstraten, ungewebten Fasersubstraten, unfaserigen, porösen Substraten und unporösen Substraten mit einer texturierten oder unebenen Oberflächenstruktur ausgewählt ist.

18. Das Verfahren nach Anspruch 17, wobei der Schritt (a) das Trocknen oder Aushärten der ersten Überzugsschicht oder des ersten Satzes von Überzugsschichten (P) umfasst, um sie resistent zu Berührungen zu machen.

19. Das Verfahren nach Anspruch 18, wobei das Trocknen oder Aushärten durch ein Verfahren durchgeführt wird, das aus UV-Härten, Elektronenstrahlhärten, Oxypolymerisationstrocknen, physikalischem Trocknen und Kombinationen davon ausgewählt wird.

20. Das Verfahren nach einem der Ansprüche 17 bis 19, wobei die erste Überzugsschicht (P) oder zumindest die oberste Schicht des ersten Satzes von Überzugsschichten (P) durch ein Druckverfahren aufgebracht wird, das aus dem Tintenstrahldruck, Offsetdruck, Flexodruck, Tiefdruck, Siebdruck, Buchdruck, Abziehbilddruck, Tampondruck und Rollenbeschichten ausgewählt wird.

21. Das Verfahren nach einem der Ansprüche 17 bis 20, wobei Informationen, wie beispielsweise eine Seriennummer oder Personalisierungsinformationen, in die erste Überzugsschicht (P) oder mindestens eine des ersten Satzes von Überzugsschichten (P) durch ein Verfahren zum Drucken von variablen Informationen, vorzugsweise durch Lasermarkierung, eingeschrieben werden.

22. Das Verfahren nach einem der Ansprüche 17 bis 21, wobei die Partikeln (F) in der zweiten Überzugsschicht oder dem zweiten Satz von Überzugsschichten (I) von magnetischen Pigmentflocken, vorzugsweise von optisch reflektierenden magnetischen Pigmentflocken, gebildet werden.

23. Das Verfahren nach einem der Ansprüche 17 bis 21, wobei die Partikeln (F) in der zweiten Überzugsschicht oder dem zweiten Satz von Überzugsschichten (I) von einem optisch variablen magnetischen Pigment, vorzugsweise durch einem Dünnfilminterferenz-Pigment, gebildet werden, das entweder eine Absorberschicht/dielektrische Schicht/reflektierende magnetische Schicht oder eine Absorberschicht/dielektrische Schicht/Reflektorschicht plus eine magnetische Schichtenfolge umfasst.

24. Das Verfahren nach einem der Ansprüche 17 bis 23, wobei die erste Überzugsschicht oder der erste Satz von Überzugsschichten über einer Beschichtung aufgebracht wird, die ein cholesterisches Flüssigkristallpolymer (CFKP)-Material umfasst.

25. Das Verfahren nach einem der Ansprüche 17 bis 24, wobei die zweite Überzugsschicht oder der zweite Satz von Überzugsschichten (I), die/der die Partikel (F) umfasst, gegenüber dem Magnetfeld einer mit Indizien gravierten permanenten Magnetplatte ausgesetzt wird, während sie/er nass ist.

## Revendications

1. Un document de sécurité ou un article (D), ayant
- un substrat (S) choisi parmi des substrats fibreux tissés, des substrats fibreux non tissés, des substrats poreux non-fibreux et des substrats non poreux ayant une structure de surface texturée ou irrégulière,
- revêtu d'une première couche de revêtement ou d'un premier ensemble de couches de revêtement (P), et
- sur la première couche de revêtement ou le premier ensemble de couches de revêtement (P) une deuxième couche de revêtement ou un deuxième ensemble de couches de revêtement (I) comprenant au moins un type de particules magnétiques ou magnétisables (F), et un motif, un image ou des indices étant réalisés dans la deuxième couche de revêtement ou le deuxième ensemble de couches de revêtement (I) par une orientation des particules homogène ou localement sélective (F),
dans lequel la première couche de revêtement ou le premier ensemble de couches de revêtement (P) est/sont imprimée(s) comme des indices, des lignes, un raster, une grille, un logo, des motifs géométriques d'une manière qui agit de façon sélective sur l'image magnétique dans les zones de la superposition avec la deuxième couche de revêtement ou le deuxième ensemble de couches de revêtement (I), et
ce qui peut être obtenu par un procédé comprenant les étapes consistant à:
a) appliquer une première couche de revêtement ou un premier ensemble de couches de revêtement (P) sur au moins une partie de la surface d'un substrat (S);
b) appliquer sur la première couche de revêtement ou le premier ensemble de couches de revêtement (P) une deuxième couche de revêtement ou un deuxième ensemble de couches de revêtement (I) comprenant au moins un type de particules magnétiques ou magnétisables (F);
c) exposer la deuxième couche de revêtement ou le deuxième ensemble de couches de revêtement (I) comprenant les particules (F), tant qu'elle est humide, à au moins un champ magnétique, permettant ainsi aux particules (F) de s'orienter dans le champ magnétique ; et
d) durcir la deuxième couche de revêtement ou le deuxième ensemble de couches de revêtement (I) comprenant les particules (F), fixant ainsi de façon irréversible les particules (F) dans leurs orientations respectives.

2. Le document de sécurité ou l'article selon la revendication 1, dans lequel la première couche de revêtement ou le premier ensemble de couches de revêtement (P) présente une épaisseur de 0,3 à 50 µm.

3. Le document de sécurité ou l'article selon la revendication 1 ou 2, dans lequel la première couche de revêtement (P) ou au moins la plus haute du premier ensemble de couches de revêtement (P) est appliquée par un procédé choisi parmi l'impression à jet d'encre, l'impression offset, l'impression flexographique, l'impression en creux, l'impression par sérigraphie, l'impression en relief, l'impression de décalcomanie, l'impression de tampographie et le revêtement de rouleau.

4. Le document de sécurité ou l'article selon l'une quelconque des revendications 1 à 3, dans lequel la première couche de revêtement (P) ou au moins la plus haute du premier ensemble de couches de revêtement (P) est choisie parmi des compositions de revêtement durcissant aux UV, des compositions de revêtement durcissant par faisceau électronique, des compositions de revêtement à base de solvant, des compositions de revêtement à base d'eau, des compositions de revêtement de séchage d'oxypolymérisation et des compositions de revêtement à durcissement hybride, y compris des revêtements durcissant à base d'eau / aux UV et à base de solvant / aux UV.

5. Le document de sécurité ou l'article selon l'une quelconque des revendications 1 à 4, dans lequel la première couche de revêtement (P) ou au moins la plus haute du premier ensemble de couches de revêtement (P) est un revêtement transparent incolore.

6. Le document de sécurité ou l'article selon l'une quelconque des revendications 1 à 5, dans lequel la première couche de revêtement (P) ou au moins une du premier ensemble de couches de revêtement (P) comprend un matériau de polymère à cristaux liquides cholestériques (CLCP), présentant une couleur dépendante de l'angle de vue et réfléchissant un composant de la lumière à polarisation circulaire dans une plage de longueur d'onde déterminée.

7. Le document de sécurité ou l'article selon l'une quelconque des revendications 1 à 6, dans lequel la première couche de revêtement (P) ou au moins une du premier ensemble de couches de revêtement (P) comprend un ou plusieurs éléments dissimulés choisis parmi des colorants solubles et des pigments insolubles.

8. Le document de sécurité ou l'article selon la revendication 7, dans lequel le pigment est choisi parmi des pigments opaques blancs ou colorés, des pigments métalliques, des pigments iridescents, des pigments optiquement variables et des pigments de polymère à cristaux liquides cholestériques (CLCP).

9. Le document de sécurité ou l'article selon l'une quelconque des revendications 1 à 8, dans lequel la première couche de revêtement (P) ou au moins une du premier ensemble de couches de revêtement (P) comprend un ou plusieurs éléments dissimulés choisis parmi des composés luminescents ultraviolets, des composés luminescents visibles, des composés luminescents infrarouges, composés luminescents à conversion ascendante, des composés absorbant les infrarouges, des composés magnétiques et des marqueurs criminalistiques.

10. Le document de sécurité ou l'article selon l'une quelconque des revendications 1 à 9, dans lequel la première couche de revêtement (P) ou au moins une du premier ensemble de couches de revêtement (P) contient des informations, telles qu'un numéro de série ou une information de personnalisation étant inscrite par un procédé de l'impression d'informations variables, préférablement par le marquage au laser.

11. Le document de sécurité ou l'article selon l'une quelconque des revendications 1 à 10, dans lequel la première couche de revêtement (P) ou au moins la plus haute du premier ensemble de couches de revêtement (P) présente la propriété supplémentaire de promouvoir l'adhésion entre le substrat (S) et la deuxième couche de revêtement magnétiquement orientée ou le deuxième ensemble de couches de revêtement (I) magnétiquement orientées.

12. Le document de sécurité ou l'article selon l'une quelconque des revendications 1 à 11, dans lequel les particules (F) dans la deuxième couche de revêtement ou le deuxième ensemble de couches de revêtement (I) sont réalisées par des flocons à pigments magnétiques, préférablement par des flocons optiquement réfléchissants à pigments magnétiques.

13. Le document de sécurité ou l'article selon l'une quelconque des revendications 1 à 11, dans lequel les particules (F) dans la deuxième couche de revêtement ou le deuxième ensemble de couches de revêtement (I) sont réalisées par un pigment magnétique optiquement variable, préférablement par un pigment interférentiel en couche mince comprenant soit une séquence de couche absorbante / couche diélectrique / couche magnétique réfléchissante, soit une séquence de couche absorbante / couche diélectrique / couche de réflecteur plus une couche magnétique.

14. Le document de sécurité ou l'article selon l'une quelconque des revendications 1 à 13, dans lequel la deuxième couche de revêtement (I) ou au moins une du deuxième ensemble de couches de revêtement (I) comprend un ou plusieurs éléments dissimulés choisis parmi des composés luminescents ultraviolets, des composés luminescents visibles, des composés luminescents infrarouges, composés à conversion ascendante, des composés absorbant les infrarouges, des composés magnétiques et des marqueurs criminalistiques.

15. Le document de sécurité ou l'article selon l'une quelconque des revendications 1 à 14, dans lequel la largeur de ligne (r) du motif, image ou des indices de l'orientation magnétique est < 3 mm, préférablement < 2 mm, plus préférablement < 1 mm.

16. Le document de sécurité ou l'article selon l'une quelconque des revendications 1 à 15, qui est choisi parmi des billets de banque, des documents de valeur, des documents d'identité, des cartes, des timbres fiscaux, des étiquettes, des emballages et des produits commerciaux.

17. Un procédé de fabrication d'un document de sécurité ou d'un article selon l'une quelconque des revendications 1 à 16, comprenant les étapes consistant à :
a) appliquer une première couche de revêtement ou un premier ensemble de couches de revêtement (P) sur au moins une partie de la surface d'un substrat (S) ;
b) appliquer sur la première couche de revêtement ou le premier ensemble de couches de revêtement (P) une deuxième couche de revêtement ou un deuxième ensemble de couches de revêtement (I) comprenant au moins un type de particules magnétiques ou magnétisables (F) ;
c) exposer la deuxième couche de revêtement ou le deuxième ensemble de couches de revêtement (I) comprenant les particules (F), tant qu'elle est humide, à au moins un champ magnétique, permettant ainsi aux particules (F) de s'orienter dans le champ magnétique ;
d) durcir la deuxième couche de revêtement ou le deuxième ensemble de couches de revêtement (I) comprenant les particules (F), fixant ainsi de façon irréversible les particules (F) dans leurs orientations respectives, et
dans lequel la première couche de revêtement (P) ou au moins une du premier ensemble de couches de revêtement (P) est imprimée comme des indices, des lignes, un raster, une grille, un logo, des motifs géométriques d'une manière qui agit de façon sélective sur l'image magnétique dans les zones de la superposition avec la deuxième couche de revêtement ou le deuxième ensemble de couches de revêtement (I),
dans lequel le substrat (S) est choisi parmi des substrats fibreux tissés, des substrats fibreux non tissés, des substrats poreux non-fibreux et des substrats non poreux ayant une structure de surface texturée ou irrégulière.

18. Le procédé selon la revendication 17, dans lequel l'étape (a) consiste à sécher ou durcir la première couche de revêtement ou le premier ensemble de couches de revêtement (P) pour la rendre résistante au toucher.

19. Le procédé selon la revendication 18, dans lequel l'étape consistant à sécher ou durcir est réalisé par un procédé choisi parmi le durcissement aux UV, le durcissement par faisceau électronique, le séchage d'oxypolymérisation, le séchage physique et des combinaisons de ceux-ci.

20. Le procédé selon l'une quelconque des revendications 17 à 19, dans lequel la première couche de revêtement (P) ou au moins la plus haute du premier ensemble de couches de revêtement (P) est appliquée par un procédé d'impression choisi parmi l'impression à jet d'encre, l'impression offset, l'impression flexographique, l'impression en creux, l'impression par sérigraphie, l'impression en relief, l'impression de décalcomanie, l'impression de tampographie et le revêtement de rouleau.

21. Le procédé selon l'une quelconque des revendications 17 à 20, dans lequel des informations telles qu'un numéro de série ou des informations de personnalisation étant inscrites dans la première couche de revêtement (P) ou au moins une du premier ensemble de couches de revêtement (P) par un procédé de l'impression d'informations variables, préférablement par le marquage au laser.

22. Le procédé selon l'une quelconque des revendications 17 à 21, dans lequel les particules (F) dans la deuxième couche de revêtement ou le deuxième ensemble de couches de revêtement (I) sont réalisées par des flocons à pigments magnétiques, préférablement par des flocons optiquement réfléchissants à pigments magnétiques.

23. Le procédé selon l'une quelconque des revendications 17 à 21, dans lequel les particules (F) dans la deuxième couche de revêtement ou le deuxième ensemble de couches de revêtement (I) sont réalisées par un pigment magnétique optiquement variable, préférablement par un pigment interférentiel en couche mince comprenant soit une séquence de couche absorbante / couche diélectrique / couche magnétique réfléchissante, soit une séquence de couche absorbante / couche diélectrique / couche de réflecteur plus une couche magnétique.

24. Le procédé selon l'une quelconque des revendications 17 à 23, dans lequel la première couche de revêtement ou le premier ensemble de couches de revêtement est/sont appliquée sur un revêtement comprenant un matériau de polymère à cristaux liquides cholestériques (CLCP).

25. Le procédé selon l'une quelconque des revendications 17 à 24, dans lequel la deuxième couche de revêtement ou le deuxième ensemble de couches de revêtement (I) comprenant les particules (F) est/sont exposée, tant qu'elle est humide, au champ magnétique d'une plaque magnétique permanente aux indices gravés.
